

## UNITED STATES PATENT OFFICE

2,107,137

## DEWAXING LUBRICATING OILS

Chester E. Adams and Frederick W. Sullivan, Jr.,  
Hammond, Ind., and John A. Anderson, Chicago, Ill., assignors to Standard Oil Company,  
Chicago, Ill., a corporation of Indiana

No Drawing. Application November 1, 1933,  
Serial No. 696,242

13 Claims. (Cl. 196—19)

This invention relates to the removal of wax from oils and more particularly to the removal of mineral wax from mineral lubricating oils.

It has been the custom for many years to remove paraffin wax from lubricating oil fractions of petroleum by diluting said fractions with a light petroleum product such as naphtha, chilling the diluted oil to low temperatures to precipitate the wax, and removing the wax by filtering, settling or centrifuging. In this process, a certain amount of wax is dissolved in the diluted oil at the dewaxing temperature so that when the diluent is removed from the oil, said oil has, in general a pour point (as defined in and determined by Method D 97-30 of the American Society for Testing Materials) at least 30° F. and sometimes as much as 50° F. higher than the temperature of dewaxing. It therefore has been necessary to dewax at extremely low temperatures which necessitates expensive refrigeration and which results in decreased filtration rates because of the high viscosity of the diluted oil at the extremely low temperatures.

An object of our invention is to overcome these difficulties and to provide an efficient and economical means for removing wax from oil whereby the pour point of the finished oil is not materially higher than the dewaxing temperature and whereby extremely low dewaxing temperatures may be avoided.

A further object is to provide an improved diluent mixture and method of using the same in a dewaxing process. A further object is to provide a process which will dewax oils containing types of wax which were heretofore difficult or impossible to remove. A further object is to obtain increased filter rates and to obtain a wax in a more nearly oil-free condition and in larger yields than has heretofore been obtained. Other objects will be apparent from the following description.

This problem of providing a satisfactory dewaxing diluent has been difficult because ordinary diluents dissolve a large amount of wax, and diluents which would not dissolve wax would likewise be immiscible with oil at dewaxing temperatures. We have discovered that a wax antisolvent may be rendered miscible with a "solvent" as herein-after defined by means of certain oxygenated or halogenated compounds which we have termed "miscibility agents". We have also discovered that certain cracked petroleum products have remarkable new and unexpected properties as components in a dewaxing-diluent mixture. Our invention will be more clearly understood from the following description in which examples are described in detail.

To avoid confusion we have defined the meaning of certain terms as they are used in this specification and in the following claims.

The term "antisolvent" refers to a liquid with which wax (and to a less extent oil) is not miscible in all proportions at the desired dewaxing temperature (generally about -10° F. or between about -25° F. and about 0° F.), but which does form a one-phase substantially wax-insoluble solution with a "solvent" and oil or a "solvent", a "miscibility agent" and oil at the desired dewaxing temperature. Examples of antisolvents are methyl alcohol, ethyl alcohol, acetone, methyl ethyl ketone, ethyl formate, liquid sulfur dioxide, etc.

The term "solvent" refers to a hydrocarbon liquid that is miscible with oil in all proportions at the dewaxing temperature; examples of such liquids are benzol and more particularly the cracked petroleum compounds which will be hereinafter described and olefinic hydrocarbons.

The term "miscibility agent" may be defined as an oxygenated or chlorinated hydrocarbon completely miscible with the oil at the dewaxing temperature and capable of preventing the separation of antisolvents from oil-diluent mixtures at dewaxing temperatures; among such liquids are ethyl acetate, ethylene dichloride and iso-propyl ether.

The term "diluent" refers to the whole mixture with which the oil is diluted and comprises the solvent and antisolvent; or solvent, antisolvent and miscibility agent.

When oils are diluted with ordinary diluents and dewaxed, a large amount of wax remains in the solution. In other words, wax is dissolved by the diluent at dewaxing temperatures. If oil is mixed with an antisolvent alone, on the other hand, dewaxing is practically impossible because the oil separates from the antisolvent at the temperatures necessary for complete dewaxing. We have discovered that oxygenated and chlorinated hydrocarbons particularly those above mentioned, have the peculiar property of rendering antisolvents miscible with solvents and with the oil to be dewaxed. We do not limit ourselves to any theory or explanation of this phenomena but we have found that an antisolvent in an antisolvent-solvent-oil mixture may be effectively prevented from separating out by the simple expedient of adding a miscibility agent thereto.

In the following examples we describe the diluent mixtures used for dewaxing an overhead (distillate) Mid-Continent lubricating oil fraction having a viscosity of about 74 seconds Saybolt at 210° F. In all of the preferred embodiments we use two and one-half volumes of diluent mixture to one volume of oil, but it is to be understood that these proportions will vary considerably with the dewaxing of different oils under different conditions. From one volume to four volumes of diluent mixture to one volume of oil

is, in general, the preferred range. Oils which are more paraffinic than Mid-Continent require greater quantities of solvent and less of anti-solvent. Heavy oils generally require a higher ratio of solvent to antisolvent in a diluent mixture than do lighter ones and also require a higher ratio of diluent mixture to oil.

Our preferred solvent is a naphtha or lighter fraction obtained from the reaction products formed by a pyrolytic cracking process, preferably a vapor phase cracking process wherein gas-oil or other petroleum products are heated to temperatures of about 900-1100° F. under pressures of from 15-300 pounds per square inch. This product may be called cracked naphtha to distinguish it from the virgin or straight run naphtha produced by ordinary distillation. It contains a high proportion of olefinic hydrocarbons and it is to these that we attribute its outstanding advantages. Naphtha produced by liquid phase cracking is superior as a dewaxing diluent to ordinary naphtha but it is not as good as that produced by vapor phase cracking. This may be due to its lower content of olefinic hydrocarbons.

As one example of our improved diluent mixture we may use 25% acetone and 75% of vapor phase cracked naphtha (boiling range 160-250° F.). At dewaxing temperature of -8° F. this diluent mixture produces an oil whose pour point is +15° F.; the differential between dewaxing temperature and pour point being about 23° F. To lower this differential it would be necessary to add a greater amount of antisolvent (acetone), but this cannot ordinarily be done since mixtures containing greater amounts of acetone tend to separate into two liquid phases at dewaxing temperatures. However, the addition of a miscibility agent permits the use of more acetone and decreases this differential.

When naphtha produced by liquid phase cracking is used, the maximum acetone content is markedly lower than with a naphtha produced by vapor phase cracking and the resultant oil has an even higher pour point. Any cracked naphtha, however, produces better results than straight run naphthas and it will thus be seen that cracked naphtha, particularly those produced by vapor phase cracking are highly desirable constituents of solvent-antisolvent mixtures whether or not a miscibility agent is used. In general 15% to 60% of cracked naphtha can be used depending on the antisolvent used, the nature of the oil being dewaxed, the dewaxing temperature, the amount of diluent mixture used per unit of oil, and other factors.

We have found that when a miscibility agent is used as a third component of the diluent mixture it is possible to increase the portion of anti-solvent to a point at which substantially complete dewaxing of the oil is obtained. For example, we may use a diluent mixture containing

| Per cent                             |
|--------------------------------------|
| 65 Iso-propyl ether ----- 15         |
| Acetone ----- 35                     |
| Vapor phase cracked naphtha ----- 50 |

The use of this diluent at a dewaxing temperature of -10° F. gives a finished oil with a pour point of 0° F.—in other words, it gives a differential of less than half that of the first example and probably one-third or one-fourth that obtained by dewaxing in a simple naphtha solution.

75 It should be understood that the proportions of

the three components of high diluent mixture may vary over a considerable range. Compositions which have proved particularly useful are:

|                                      | Per cent |
|--------------------------------------|----------|
| Isopropyl ether ----- 25             | 5        |
| Acetone ----- 33                     |          |
| Vapor phase cracked naphtha ----- 42 |          |
| or                                   |          |
| Ethylene dichloride ----- 43         | 10       |
| Acetone ----- 16                     |          |
| Cracked naphtha ----- 41             | 15       |

Under various conditions the above concentrations of each of these components can be varied as much as 10% or even 15% either up or down. The miscibility agent itself may have a certain antisolvent power but its particular usefulness lies in the fact that it has the power to keep large amounts of antisolvents from separating from the diluted oil at low temperatures.

As we have pointed out we believe that the peculiar advantages of vapor phase cracked naphthas are due in large part to their high olefinic hydrocarbon content. This is borne out by the fact that olefinic hydrocarbons such as propylene, butylene, amylenes, etc., are desirable solvents and can be used together with antisolvents or antisolvents and miscibility agents. Thus, for example, from 30% to 80% of propylene, butylene, amylene or mixtures thereof can be used together with from 20% to 70% of sulfur dioxide as a dewaxing diluent under pressures sufficient to cause liquefaction of the diluent mixture.

While we have disclosed preferred embodiments of our invention in detail it is understood that we do not limit ourselves to the details hereinabove set forth except as defined by the following claims which should be construed as broadly as the prior art will permit.

We claim:

1. The process of dewaxing a wax-bearing mineral lubricating oil which comprises diluting the oil with a diluent mixture comprising substantial amounts of a wax antisolvent and a cracked petroleum naphtha, chilling the diluted oil to a low temperature, whereby the wax is caused to precipitate therefrom while the oil is retained in solution in the diluent mixture, separating the wax from the oil and diluent, and subsequently removing the diluent from the dewaxed oil.

2. The process of dewaxing a wax-bearing mineral lubricating oil which comprises diluting the oil with a diluent mixture comprising substantial amounts of a wax antisolvent, a cracked petroleum naphtha and a miscibility agent, chilling the diluted oil to a low temperature, whereby the wax is caused to precipitate therefrom while the oil is retained in solution in the diluent mixture, separating the wax from the oil and diluent, and subsequently removing the diluent from the dewaxed oil.

3. The process of dewaxing mineral lubricating oils according to claim 1 wherein the petroleum naphtha is produced by a vapor phase cracking process.

4. The process of dewaxing lubricating mineral oils according to claim 1 wherein acetone is employed as the antisolvent in the diluent mixture.

5. The process of dewaxing lubricating mineral oils according to claim 2 wherein iso-propyl ether is employed as the miscibility agent in the diluent mixture.

6. The process of dewaxing lubricating mineral

oils according to claim 2 wherein the diluent mixture employed is comprised of cracked petroleum naphtha, acetone and iso-propyl ether.

7. The process of claim 1 wherein the anti-solvent is methyl ethyl ketone.

8. The process of claim 1 wherein the anti-solvent is sulfur dioxide.

9. The process of claim 2 wherein the anti-solvent is acetone.

10. The process of claim 2 wherein the anti-solvent is methyl ethyl ketone.

11. The process of claim 2 wherein the anti-solvent is sulfur dioxide.

12. The process of claim 2 wherein the miscibility agent is ethylene dichloride.

13. The process of claim 2 wherein the cracked petroleum naphtha is produced by vapor phase cracking.

CHESTER E. ADAMS.

FREDERICK W. SULLIVAN, JR.

JOHN A. ANDERSON.

10

CERTIFICATE OF CORRECTION.

Patent No. 2,107,137.

February 1, 1938.

CHESTER E. ADAMS, ET AL.

It is hereby certified that error appears in the printed specification of the above numbered patent requiring correction as follows: Page 2, second column, line 56, claim 2, after "agent" and before the comma insert the words for antisolvent and oil; and that the said Letters Patent should be read with this correction therein that the same may conform to the record of the case in the Patent Office.

Signed and sealed this 15th day of March, A. D. 1938.

(Seal)

Henry Van Arsdale,  
Acting Commissioner of Patents.

oils according to claim 2 wherein the diluent mixture employed is comprised of cracked petroleum naphtha, acetone and iso-propyl ether.

7. The process of claim 1 wherein the anti-solvent is methyl ethyl ketone.

8. The process of claim 1 wherein the anti-solvent is sulfur dioxide.

9. The process of claim 2 wherein the anti-solvent is acetone.

10. The process of claim 2 wherein the anti-solvent is methyl ethyl ketone.

11. The process of claim 2 wherein the anti-solvent is sulfur dioxide.

12. The process of claim 2 wherein the miscibility agent is ethylene dichloride.

13. The process of claim 2 wherein the cracked petroleum naphtha is produced by vapor phase cracking.

CHESTER E. ADAMS.

FREDERICK W. SULLIVAN, JR.

JOHN A. ANDERSON.

10

CERTIFICATE OF CORRECTION.

Patent No. 2,107,137.

February 1, 1938.

CHESTER E. ADAMS, ET AL.

It is hereby certified that error appears in the printed specification of the above numbered patent requiring correction as follows: Page 2, second column, line 56, claim 2, after "agent" and before the comma insert the words for antisolvent and oil; and that the said Letters Patent should be read with this correction therein that the same may conform to the record of the case in the Patent Office.

Signed and sealed this 15th day of March, A. D. 1938.

(Seal)

Henry Van Arsdale,  
Acting Commissioner of Patents.

CERTIFICATE OF CORRECTION.

Patent No. 2,107,137.

February 1, 1938.

CHESTER E. ADAMS, ET AL.

It is hereby certified that error appears in the printed specification of the above numbered patent requiring correction as follows: Page 2, second column, line 56, claim 2, after "agent" and before the comma insert the words for antisolvent and oil; and that the said Letters Patent should be read with this correction therein that the same may conform to the record of the case in the Patent Office.

Signed and sealed this 15th day of March, A. D. 1938.

(Seal)

Henry Van Arsdale,  
Acting Commissioner of Patents.